

H. C. EGERTON.  
PROCESS OF MAKING EXTRUDED FIBROUS SHAPES.  
APPLICATION FILED APR. 28, 1919.

1,370,800.

Patented Mar. 8, 1921.



### Inventor

Henry C Egerton  
By his Attorney  
Harry Duncan

# UNITED STATES PATENT OFFICE.

HENRY C. EGERTON, OF RIDGEWOOD, NEW JERSEY.

## PROCESS OF MAKING EXTRUDED FIBROUS SHAPES.

1,370,800.

Specification of Letters Patent.

Patented Mar. 8, 1921.

Application filed April 28, 1919. Serial No. 292,941.

To all whom it may concern:

Be it known that I, HENRY C. EGERTON, a citizen of the United States, and resident of Ridgewood, Bergen county, New Jersey, have made a certain new and useful Invention Relating to Processes of Making Extruded Fibrous Shapes, of which the following is a specification, taken in connection with the accompanying drawing, which forms part of the same.

This invention relates especially to processes of making tubes, rods, sheets or other extruded shapes from material which may contain suitable proportions of incorporated cured phenolic condensation cementing material, such as bakelite, condensite or redmanol compositions which may be present to the extent of thirty or sixty per cent. in the finished article, dependent, of course, on the portions of fibrous and inert coloring or other special material contained in these cementing compositions. Many suitable forms of fibrous material may be used for this purpose, such as cotton or flax fiber in various forms, such, for example, as cotton batting or wadding which may sometimes be advantageously formed of special cotton fiber material which is preferably of substantially uniform length and for some such extruded articles may with advantage be of relatively short length fiber, such as a quarter of an inch long more or less. In some cases also suitable proportions of other fibrous material may be used, such as Kraft paper pulp, rag stock, or the like, and in some cases it is advantageous to subject cotton or refined flax fiber to a beating process as in a paper pulp beater or refining engine to reduce the fiber to the desired relatively short uniform length and to separate the fibers to the desired extent for the incorporation therewith of the phenolic condensation cementing material desired which may be effected in various ways to preferably effect a substantially uniform incorporation of the fiber and other material before the extrusion of the material in the plunger or screw extrusion press of any suitable character where it may be subjected to the desired high extrusion pressure under con-

trolled heating conditions so as to form a substantially uniform fibrous extruded shape which is sufficiently cured to retain its shape with or without subsequent curing. It is usually desirable to have the impregnated or cemented fibrous material in partly cured condition before it is subjected to the extrusion step and it is also advantageous to have it preliminarily compressed so that substantially all air or similar material is driven out and air bubbles or weakened portions avoided in the finished article. The impregnated or cemented fibrous material may for this purpose be compressed under moderate heat to high pressure and this may advantageously be done under such conditions that a preliminary partial vacuum treatment of the material serves to withdraw at least a large part of the air therefrom before the compression thereof so that in this way blocks, sheets or strips of such compressed partly cured cemented fibrous material may be formed for feeding continuously or intermittently into the screw or other extruding presses. For many purposes it is desirable to have the material before extrusion cured or solidified to at least a very considerable extent so that it is in a substantially solidified but weldable or unitable condition so that it may be united thoroughly and strongly under the high extrusion pressure and for this purpose suitable softening or uniting agents may be incorporated with the cementing-material, such as a few per cent. of anilin or other oily or softening uniting agent which makes it possible to unite severed portions of the material under heat at considerable pressure even after the curing has reached quite an advanced stage.

The impregnated or cemented fibrous material with or without such preliminary compression may be forced under proper heat and pressure through an extrusion die so as to form a continuous stream of highly compressed extruded material which may be heated and further cured while in this condition and before the extrusion pressure is completely released so that a completely solidified or cured extruded article may be produced in this way. For many purposes

a solid or hollow mandrel may be arranged within the extrusion die so as to form a hollow extruded article in connection, if desired, with one or more cores, wires, or other members which may be fed into the same during the extrusion thereof. In some cases also either with or without such a metallic wire or core, impregnated fibrous material of this character may be extruded either in side or outside of a sheath of rubber, gutta percha, or other material which is desirable for some classes of electrical work.

The drawing shows in a somewhat diagrammatic way various forms of apparatus for carrying out this process, and

Figure 1 is a vertical section through an extruding press which may be used.

Fig. 2 is a perspective view of a blank or block of material for use in this connection; and

Fig. 3 is a sectional view through a curing chamber which may be used in some cases for subsequent curing of the extruded articles.

Where little or no inert coloring or other special material is used the fibrous composition may comprise some forty to sixty per cent. of dried bakelite varnish or similar somewhat cured or combined phenolic condensation cementing material incorporated with sixty to forty per cent. of relatively short uniform cotton fiber or other suitable fibrous material. This incorporation may be effected in any suitable way so as to preferably effect the substantially uniform incorporation of the components. For some purposes beaten, clipped or otherwise prepared raw cotton fiber of good quality may be formed into sheets of wadding or batting and then sprayed or more or less immersed in warmed condition, preferably after inclosing the same between thin fabric layers to facilitate handling in suitable bakelite varnish compositions which may advantageously in many cases contain relatively small proportions of the solvents used with the phenolic condensation cementing material. The solvent promotes the uniform penetration of the cementing material throughout the fibrous material with which it is incorporated and the individual fibers can thus be readily coated or united with the material so as to secure a more uniformly cemented fibrous composition which is advantageous for most extruded articles. In some cases instead of spraying or immersing sheets of such pure fibrous material the incorporation may be effected in suitable mixing apparatus, such as kneading ma-

chines of the Werner-Pfleiderer type. Under these conditions the material may be somewhat warmed which minimizes the amount of solvent necessary and this may be still further minimized by using relatively uncured phenolic condensation ce-

menting material for incorporation with the fibrous components in the first instance, the preliminary curing changes being effected, if desired, by the heat used during the incorporating or mixing processes. Of course for some purposes relatively short fiber may be used to a greater or less extent and sulfate or Kraft pulp may be used preferably after being preliminarily heated to three or four hundred degrees and cooled at least to some extent before being incorporated with the phenolic condensation cementing material which seems to facilitate the incorporation of the phenolic condensation material with the ultimate wood fibers of this or other suitable wood pulp material. Of course when the thorough incorporation of the components has been effected this cemented or impregnated fibrous material may be suitably dried under reduced pressure, if desired, so as to remove any volatile components or solvent elements and then formed into sheets, rods, blocks or other blanks for use in this process.

It is usually advantageous to remove the entrained air from such cemented fibrous material and also in most cases to press and partly cure the same before the extruding operation, and for this purpose the cemented or impregnated fibrous material may be compressed preferably after a vacuum treatment to remove the air so as to form compressed blanks of suitable shape and size so that, for instance, a cylindrical blank 22 may be formed of suitable fibrous material of this character and subjected to the desired curing treatment before or after being compressed into this form so that the material approaches sufficiently to the solid moderately or completely cured condition, so that a comparatively short heat treatment is sufficient to give the desired strength and rigidity to the extruded article either during or after the extruding step. Fig. 1 shows a form of plunger extruding press which may be used for making such extruded fibrous shapes or articles and the press body 1 may be formed with a cylindrical bore 2 of such size as to receive the compressed blanks 22 of partly cured fibrous material which may then be compressed by the hydraulic or other plunger 3 fitting fairly tightly within this bore or chamber. The extrusion chamber may be formed with a shaped discharge end 27 having a more or less tapering throat 5 of such size and shape as corresponds to the article or extruded shape to be formed and this may be conveniently effected by using a removable die 4 which may be screwed into the body or chamber of the press, so that the highly compressed material may be forced into the contracting throat and form a stream of extruded material, such as 24, of the desired size and shape. It is of course under-

stood that in some cases where a tubular or other hollow article is desired an internal mandrel 9 may be used within the die and this may be formed on a removable support 5 7 having a tapered portion 8 coöperating with the throat of the extrusion die and a threaded end 6 on this member may be screwed into the opposite end of the press body so that the mandrel coöperates with 10 the extruding passage in the die. Of course the mandrel or extruding die passage or both may be given special shapes to form correspondingly shaped extruded sections and in this way square sectioned tubes or 15 corrugated tubes or gear pinions or other irregular shapes may be conveniently and accurately formed of such fibrous material which by varying the proportions and character of the fibrous material contained may 20 be given corresponding strength, toughness and rigidity.

It is desirable where the cemented fibrous material is in partly cured condition when it is supplied to the extrusion press to heat 25 it to at least a moderate degree before it is forced through the throat of the extrusion die and at about the time the material enters this extrusion passage it may advantageously be heated to a considerably greater 30 temperature, such as 300° to 350° Fahrenheit, or in some cases to still higher temperatures which effect a correspondingly quicker and more complete cementing and 35 curing action on the fibrous material especially under the high extrusion pressure used which may be a number of thousand pounds per square inch in many cases. This heating of the extruded material may 40 be effected by having the extruding die 10 of considerable length and an extruding passage a number of feet long may advantageously be used where a considerable curing action is to be effected during this part of the process. By the use of suitable heating 45 elements around or in connection with the extruding die, such, for example, as the steam or other heating pipes 15 which may have the connections 16, 17, one or more feet of this extruding passage may be heated 50 to quite high temperatures, such as 400° to 500° Fahrenheit or more, although char- 55 ring and undesirable transformation of the material should of course be avoided; such high curing heats effectively cure, cement and unite the fibrous material during this 60 part of the process while it is still subjected to considerable pressure. Where such relatively high temperatures are used it is usually desirable to at least partly cool the heated 65 extruded material before the extrusion pressure is completely released and for this purpose the discharge end of the extrusion passage may be cooled by any suitable means, such, for example, as brine or other cooling pipes 18, arranged or coiled around

any desired length of the discharge end of the extrusion passage and having inlet and outlet connections 19, 20. Suitable heat insulating material, such as 26, may of course be arranged around the extrusion passage 70 so as to prevent heat transfer therefrom.

The extruded article 24 may be kept under suitable longitudinal compression during the extrusion process by regulating its movement past the discharge end of the 75 extrusion die or passage and this may be effected by regulating the size of this part of the passage or by arranging suitable drag plates or members, such as 12, which may have projections or portions fitting within 80 the annular recess 11 in the end of the extrusion die. By the use of a tapered or conical compression member 13 which may have a cylindrical threaded portion 14 co-operating with these drag members 12 their 85 discharge ends may be forcibly compressed or brought together so as to frictionally engage the extruded article 24 to a sufficient extent to prevent undesirable release of 90 pressure thereon and prevent development 95 of gas or expansion action when relatively high curing heats are used at various parts of the extrusion passage or process. Of course, when the hydraulic or other plunger 3 nears the bottom of the extrusion chamber 100 it may be quickly withdrawn and another blank or block 22 of the compressed partly cured fibrous material such as is shown in Fig. 2 may be inserted in the chamber and compressed beneath the plunger so as to be 105 gradually forced out through the extrusion die when the other material 23 has been discharged. By having the cemented or im- 110 pregnated fibrous material in partly or substantially cured cemented condition when it is supplied to the extrusion press of the plunger or continuous screw type it is suffi- 115 ciently consistent so that under the moderate temperatures used in the main extrusion chamber as determined by the heating jets or other heating means 21 the incorporated phenolic condensation cementing material does not tend to flow through or past the fibrous material to an undesirable extent, especially where relatively short uniform 120 fiber is used. Thus sufficient uniformity of character of the extruded material may be secured for many types of insulating or other articles which may be readily and conveniently formed of accurate cross-sec- 125 tion and polished surfaces, if desired.

It is sometimes desirable to subsequently cure the extruded articles in continuous lengths or separated pieces and for this purpose they may be cured at the desired 125 temperature in air or steam chambers under pressure in some cases or by immersing them in oily or waxy heating mediums by which suitable waxy or other coatings may be conveniently applied thereto which is 130

desirable for some forms of electrical bushings or insulating tubes of this general character. Fig. 3 shows a pressure curing chamber which may be used in connection with an extrusion press for producing lengths of such fibrous material. The chamber 30 may be formed of strong sheet steel or other material and may have an inlet end or portion 33 having a threaded connection 32 with the end 31 of the extrusion die which under these conditions need not always be of such length or heated and cooled to such an extent as described in connection with the Fig. 1 extrusion apparatus. The extruded article or shape 24 may thus be delivered into the chamber 30 which may be heated to the desired curing temperature and kept under considerable pressure by steam or other heating fluid which may be supplied through the connection 45 formed, if desired, in the end plate 43 removably secured to the chamber as by the bolts 44. In some cases it is desirable to successively cut off lengths of the extruded material as it enters the chamber, and for this purpose a cutting device of any suitable character may be installed in connection with or inside the chamber so as to cut off any suitable lengths 25 of the extruded rod, tube, strip or shape which may then be further cured within the chamber before the extrusion pressure has been reduced to atmospheric pressure. A form of cutter which is diagrammatically indicated in this connection may comprise the steel disk 36 formed with a series of cutting apertures 37 in its periphery and revolvably mounted on a stem 38 projecting through a packed or other gland in the end 40 of the curing chamber. A handle or lever 39 on this stem may be used to quickly swing the cutting disk across the advancing extruded article so that a narrow portion of the disk cuts through the extruded material before another adjacent opening is reached in the disk which allows another length of material to enter the chamber and be cut off in turn. The length of the material cut off in this way may be controlled in any suitable manner either by visually observing the length of material within the chamber and manually operating the cutting device in accordance therewith or by electrical or other automatic means which may be used in this connection. As indicated an observation opening 42 may be formed in the chamber and covered by a glass or other transparent member 40 in the frame 41. When sufficient material has accumulated in such a curing chamber it may be removed from the press or the material taken out of the chamber. It is, however, desirable in some cases to continue the curing of the lengths of the material for a considerable time and for this purpose for in-

stance when a new disk or blank of fibrous material is being inserted in the extruding chamber of the press the entrance portion 33 of the curing chamber may be closed as by the cutting or gate valve 35 which may be forced down within its casing 34 so as to sever the partial length of material 24 and then hermetically seal the curing chamber which may then be released from the die 31 with which it may have any suitable screw connection and another similar curing chamber applied to receive the extruded lengths which are produced by the press as soon as the recharging thereof has been completed preferably within a very short time to minimize local over-curing of the material within the heated extrusion passages, etc. It is not, however, necessary in all cases to completely cure the extruded material and it is advantageous for some purposes to have the extruded and shaped material left in such partly cured condition that the extruded tubes, rods or other articles may be heated and bent or otherwise reshaped after being extruded or in connection with the extrusion process which facilitates their use in manufacturing certain classes of chemical or electrical apparatus or for other purposes. After such bending, shaping or uniting treatment the partly cured material may then be still further or more completely cured by suitable heat under pressure, if desired, so as to give the completely shaped articles greater strength and security of union in various parts. While for electrical insulating purposes it is usually desirable to have relatively pure mixtures of cotton or other suitable cellulose fiber and bakelite or other phenolic condensation cementing material, yet for some purposes more or less coloring or inert filling or other special material may be used in such extruding compositions to more or less replace at least part of the fibrous material used and the material preferably after being properly incorporated and preferably more or less compressed and partly cured may be extruded into the desired shape and simultaneously cured to a greater or less extent in the manner described. In some cases fibrous or other asbestos may be used instead of the cellulose fiber referred to and for some special purposes fibrous material may be substantially omitted or replaced by powdered or other inert filling or coloring materials to form extruding compositions containing considerable proportions, such as 30 to 60 per cent, more or less of phenolic condensation cementing material.

This invention has been described in connection with a number of illustrative embodiments, forms, materials, proportions, conditions of temperature, pressure, time and other treatment and nature and order

of steps, to the details of which disclosure the invention is not of course to be limited, since what is claimed as new and what is desired to be secured by Letters Patent is 5 set forth in the appended claims:

1. The process of forming tubes or other extruded shaped lengths of fibrous material containing incorporated cured phenolic condensation cementing material which comprises thoroughly incorporating with relatively short uniform length fibrous material phenolic condensation cementing material to the extent of at least thirty per cent. by weight thereof to form cemented fibrous material, compressing said fibrous material to remove air therefrom and forming compressed blanks thereof and partly curing such cemented fibrous material, heating and forcing the same through an extruding die 10 having a central mandrel to form a hollow extruded article around said mandrel, heating such shaped extruded hollow article and cooling the same while controlling its longitudinal movement and completing the curing of the phenolic condensation cementing material in the extruded article.
2. The process of forming tubes or other extruded shaped lengths of fibrous material containing incorporated cured phenolic condensation cementing material which comprises incorporating with fibrous material phenolic condensation cementing material to the extent of at least thirty per cent. by weight to form cemented fibrous material, compressing said fibrous material to remove air therefrom and forming compressed blanks thereof and partly curing such cemented fibrous material, heating and forcing the same through an extruding die having a central mandrel to form a hollow extruded article around said mandrel, heating such shaped extruded hollow article and cooling the same while controlling its longitudinal movement.
3. The process of forming extruded shaped lengths of fibrous material containing incorporated cured phenolic condensation cementing material which comprises incorporating with fibrous material phenolic condensation cementing material to the extent of at least thirty per cent. by weight thereof to form cemented fibrous material, compressing said fibrous material to remove air therefrom and forming compressed blanks thereof and partly curing such cemented fibrous material, heating and forcing the same through an extruding die having a central mandrel to form extruded article, heating such shaped extruded article and cooling the same while controlling its longitudinal movement.
4. The process of forming rods, tubes or other extruded shaped lengths of fibrous material containing incorporated cured phenolic condensation cementing material which

comprises thoroughly incorporating relatively short length fibrous material with phenolic condensation cementing material to form cemented fibrous material, compressing said fibrous material to remove air therefrom 70 and forming compressed blanks thereof and partly curing such cemented fibrous material, heating and forcing the same through an extruding die having a central mandrel to form a hollow extruded article around said mandrel, heating said shaped extruded article and cooling the same while controlling its longitudinal movement and completing the curing of the phenolic condensation cementing material in the extruded 80 article.

5. The process of forming rods, tubes or other extruded shaped lengths of fibrous material containing incorporated partly cured phenolic condensation cementing material which comprises thoroughly incorporating fibrous material with phenolic condensation cementing material to form cemented fibrous material, partly curing such cemented fibrous material, heating and forcing the same through an extruding die having a central mandrel to form a hollow extruded article around said mandrel.

6. The process of forming rods or other extruded shaped lengths of fibrous material 95 containing incorporated partly cured phenolic condensation cementing material which comprises thoroughly incorporating fibrous material with phenolic condensation cementing material to form cemented fibrous material, partly curing such cemented fibrous material, heating and forcing the same through an extruding die to form an extruded article.

7. The process of forming extruded 105 shaped lengths of fibrous material containing incorporated cured phenolic condensation cementing material which comprises incorporating with fibrous material phenolic condensation cementing material to the extent of at least forty per cent. by weight thereof to form impregnated fibrous material, partly curing such fibrous material, heating and extruding the same, a shaped extruded article, heating said shaped extruded article and cooling the same while controlling its longitudinal movement and substantially completing the curing of the phenolic condensation cementing material in the extruded article.

8. The process of forming extruded shaped lengths of fibrous material containing incorporated cured phenolic condensation cementing material which comprises incorporating with fibrous material phenolic condensation cementing material to form impregnated fibrous material, partly curing such fibrous material, heating and extruding the same, a shaped extruded article, heating said shaped extruded article 125

130

while controlling its longitudinal movement and substantially completing the curing of the phenolic condensation cementing material in the extruded article.

5 9. The process of forming extruded fibrous articles containing partly cured phenolic condensation cementing material which comprises forming compressed cemented fibrous material containing thirty to sixty per cent. 70  
10 by weight of partly cured incorporated phenolic condensation cementing material, heating and extruding such compressed cemented fibrous material and cooling the resulting extruded article before its complete 75  
15 release from pressure.

10. The process of forming extruded fibrous articles containing partly cured phenolic condensation cementing material which comprises forming compressed fibrous material containing partly cured incorporated phenolic condensation cementing material, heating and extruding such compressed cemented fibrous material and cooling the resulting extruded article before its complete 80  
20 release from pressure.

11. The process of forming extruded fibrous articles containing partly cured phenolic condensation cementing material which comprises forming compressed fibrous material containing partly cured incorporated phenolic condensation cementing material, heating and extruding such compressed cemented fibrous material. 85  
30

12. The process of forming extruded articles of fibrous material containing partly cured phenolic condensation cementing material which comprises forming short length fiber material containing over thirty per cent. by weight of partly cured phenolic 90  
40 condensation cementing material, heating and extruding such fiber material and cooling the resulting extruded article before its release.

13. The process of forming extruded articles of fibrous material containing partly cured phenolic condensation cementing material which comprises forming fiber material containing partly cured phenolic condensation cementing material, heating and 95  
50 extruding such fiber material and cooling the resulting extruded article before its release.

14. The process of forming extruded articles of fibrous material containing partly cured phenolic condensation cementing material which comprises forming compressed cemented fibrous material containing incorporated partly cured weldable phenolic condensation cementing material, heating and 105  
60 extruding such compressed cemented fibrous material and cooling the resulting extruded article before its release.

15. The process of forming extruded articles of fibrous material containing partly cured phenolic condensation cementing ma- 110  
65

terial which comprises forming cemented fibrous material containing incorporated cured weldable phenolic condensation cementing material, heating and extruding such compressed cemented fibrous material. 70

16. The process of forming tubes or other extruded shaped lengths of fibrous material comprising incorporated cured phenolic condensation cementing material and fibrous material, which comprises compressing such 75  
fibrous material to remove air therefrom and forming compressed blanks thereof and partly curing such material, heating and forcing such material through an extruding die having an inner mandrel to form a hollow extruded article around said mandrel, heating said shaped extruded article and cooling the same while controlling its longitudinal movement and completing the curing of the phenolic condensation cementing 80  
85 material in the extruded article.

17. The process of forming tubes or other extruded shaped lengths comprising incorporated cured phenolic condensation cementing material, which comprises compressing 90  
such material to remove air therefrom and forming compressed blanks thereof and partly curing such material, heating and forcing such material through an extruding die having an inner mandrel to form a hollow extruded article around said mandrel, heating said shaped extruded article and cooling the same while controlling its longitudinal movement. 95

18. The process of forming extruded 100 shaped lengths comprising incorporated cured phenolic condensation cementing material, which comprises compressing such material and forming compressed blanks thereof and partly curing such material, heating and forcing such material through an extruding die to form an extruded article, heating said shaped extruded article and cooling the same while controlling its longitudinal movement. 105  
110

19. The process of forming rods, tubes or other extruded shaped lengths of material comprising at least thirty per cent. of incorporated cured phenolic condensation cementing material, which comprises forming and partly curing such material, heating such material and forcing the same through an extruding die having an inner mandrel to form a hollow extruded article around said mandrel, heating said shaped extruded article and cooling the same while controlling its longitudinal movement. 115  
120

20. The process of forming extruded shaped lengths of material comprising at least thirty per cent. of incorporated cured phenolic condensation cementing material, which comprises forming and partly curing such material, heating such material and forcing the same through an extruding die to form an extruded article, heating said 125  
130

shaped extruded article and cooling the same while controlling its longitudinal movement.

21. The process of forming extruded shaped lengths of material comprising at least thirty per cent. of incorporated phenolic condensation cementing material,

which comprises forming and partly curing such material, forcing such material through an extruding die to form an extruded article, heating said shaped extruded article and further curing the same before releasing the same from pressure.

HENRY C. EGERTON.